

# UNITED STATES PATENT OFFICE.

GEORGE L. COLLORD, OF PITTSBURGH, PENNSYLVANIA.

## TREATING ORES.

1,343,250.

Specification of Letters Patent. Patented June 15, 1920.

No Drawing.

Application filed May 9, 1919. Serial No. 296,031.

*To all whom it may concern:*

Be it known that I, GEORGE L. COLLORD, residing at Pittsburgh, in the county of Allegheny and State of Pennsylvania, a citizen 5 of the United States, have invented or discovered certain new and useful Improvements in Treating Ores, of which improvements the following is specification.

It is a peculiarity of some ores found in 10 certain parts of the Mesaba region and also in other parts of the country that they contain a high percentage of moisture and are so lean that nearly all the moisture must be removed to raise the contained ore to 15 a commercially workable percentage, *i. e.*, about fifty per cent. It has been attempted to dry out these ores to bring the ore content up to a minimum percentage justifying reduction in a furnace but it was found 20 that when the moisture had been reduced to seven per cent., the ore was extremely dusty, in which condition it cannot be transported or used in a blast furnace.

It has been found that if an oleaginous 25 material such as tar or some form of petroleum, be added to ores either before or while being dried, the oil will form a protective coating on all the particles of ore and that when so coated, the percentages of 30 moisture can be reduced to or below three per cent. (3%) without the ore being disintegrated in the drying.

In lieu of applying the tar or oil prior to

or while the moisture is being reduced to the desired percentage, as described and 35 claimed in an application, Serial Number 296030, filed of even date herewith, the ore may be subjected to the drying operation in any suitable form or construction of drier, and after the moisture has been reduced to the desired percentage, *e. g.*, to three or two and one-half—(3 or  $2\frac{1}{2}$ )—per cent., the tar or oil is mixed with the dried ore. It has been found, however, that as there is practically no moisture present to facilitate 45 or promote the spreading of the oil or tar over the surfaces of the particles, a larger percentage of oil than that required for the method described in the application above referred to, must be employed, as for 50 example, eight to ten per cent. more or less. It has been found that by the addition of the oleaginous material, the particles of dust will collect and adhere together forming small grains and entirely free from dust. 55

I claim herein as my invention:

The method herein described of treating moist ore, which consists in reducing the percentage of moisture in the ore, and mixing with the ore thus treated an oleaginous 60 material adapted to cause an agglomeration of the fine particles of the ore.

In testimony whereof, I have hereunto set my hand.

GEO. L. COLLORD.